

## UNITED STATES PATENT OFFICE

2,516,664

HYPOCHLORITE BLEACHING OF GROUND  
WOOD

Daniel O. Adams and George B. Hughey, Covington, Va., assignors to West Virginia Pulp and Paper Company, New York, N. Y., a corporation of Delaware

No Drawing. Application October 16, 1944,  
Serial No. 558,952

5 Claims. (Cl. 8—105)

1

Our present invention relates to improvements in the bleaching of ground wood, more especially ground oak and other ground woods such as chestnut, chestnut oak, maple, etc., which contain a substantial amount of tannin and other natural color bodies.

In recent years much study has been given to the bleaching of ground wood. Usually and especially for the manufacture of newsprint, ground wood is not bleached. However, the desirable printing characteristics of paper containing a large proportion of ground wood have led to proposals for its use in high grades of paper such as magazine, book paper and the like. In many instances a base ground wood sheet or one containing a substantial proportion of ground wood is coated with a suitable coating composition. However, to be successful the ground wood must have a reasonably good color of substantial permanence, otherwise only a slight proportion of it may be used in the furnish; or if used in substantial proportion in the base sheet an undesirably heavy coat must be given it in order to have a final product of acceptable brightness.

Prior to our discovery the most successful attempts to bleach ground wood have been those involving the use of sodium peroxide. We have discovered, however, that under properly controlled conditions even superior results may be had by hypochlorite bleaching. In applying our improved hypochlorite method to the bleaching of ground hard woods, as for example oak and other woods containing appreciable amounts of tannin, it is not practicable to obtain as bright a pulp as with ground spruce, for example. We have discovered, however, that the ground hard woods such as oak, chestnut, etc., may be made to yield a bleached pulp of comparable brightness with bleached ground spruce or poplar by subjecting the ground hard wood to a preliminary dilute caustic extraction whereby to remove certain of the incrustations and color bodies associated with the fiber, which extraction is directly followed, after washing, by the hypochlorite bleach.

After the hypochlorite bleach is had, the brightness may be further increased by the use of a moderate excess of an anti-chlor, preferably sulfurous acid.

Our invention will be best understood by ref-

2  
erence to the following detailed examples illustrative thereof.

*Example I.—Without caustic extraction*

5 A slurry of ground wood prepared from red oak containing 15.2 grams of oven dried (O. D.) pulp at 5% consistency was heated to 90° F. To this slurry 0.5 grams of NaOH was added. A volume of calcium hypochlorite solution containing 1.5 10 grams available chlorine was added with agitation, given an initial pH of 10.1. Thereafter during the bleach the pH was maintained between 10 and 10.5 by additions of NaOH solution as required. The bleach was permitted to proceed to 15 exhaustion of the hypochlorite, which required twenty minutes. As soon as exhaustion had occurred 1.5 grams SO<sub>2</sub> were added and the mixture allowed to stand ten minutes. The pulp was thickened on a Buechner funnel and thoroughly 20 washed. This bleaching increased the brightness of the pulp from 43.1% to 57.0% as determined by the General Electric reflection meter using a No. 1 filter. When the hypochlorite was increased to 2.25 grams available chlorine (i. e., 25 15% based on the O. D. pulp) the exhaustion period was found to be sixty minutes and a final brightness of 61.2 resulted, with other conditions having remained the same.

*Example II.—With caustic extraction*

30 A 1745 gram sample of ground wood prepared from red oak was treated with 35 grams NaOH in sufficient solution to give a final concentration of 1 gram per liter. This resulted in a pulp slurry of approximately 5% consistency (O. D. basis). The temperature was maintained at 77° F. and at the end of one hour the pulp slurry was thickened on a filter and thoroughly washed.

35 The pulp from the foregoing extraction was then dispersed in water, and sufficient calcium hypochlorite solution to contain 175 grams available chlorine (equal to 10% of the weight of the unbleached pulp) was added to the slurry. The pH was maintained between 10 and 10.5 throughout the bleach. After the bleach liquor was 40 added, the consistency of the slurry was 5.0% O. D. and the temperature 95° F. The bleach was allowed to proceed until the chlorine was practically exhausted, and then 168 grams of SO<sub>2</sub> were added. After ten minutes the pulp was 45

thickened on a filter and thoroughly washed. The resulting pulp had a brightness of 67.5 as determined with the General Electric reflection meter.

When the strength of the caustic extraction solution was increased to 5 grams per liter, a final brightness of 71.8 was obtained, other conditions having remained substantially the same.

In the caustic extraction step temperature has not been found to be critical. At 65° F. substantially the same results were obtained as at 140° F. In general no increased benefits were had by increasing the amount of sodium hydroxide beyond 10% based on the dry weight of the pulp. In carrying out the hypochlorite bleach, brightening of the pulp occurred at a pH slightly above 7, with optimum results between 10.0 and 11.5. Variation in pulp consistency in the hypochlorite bleaching stage between 5 and 10% O. D. was without noticeable effect in the result. However, the brightness of the pulp increased with the concentration of hypochlorite until 10% to 15% available chlorine on unbleached dry pulp basis was added. Further increases in the quantity of bleach added were found to cause a decrease in brightness of resulting pulp. In lieu of calcium hypochlorite other compounds yielding hypochlorite ions may be used, e. g., the alkali metal hypochlorites and other alkaline substances yielding hydroxyl ions may be used in the extraction step, such as sodium carbonate, trisodium phosphate, sodium sulfide, sodium sulfite, sodium silicate, etc., as well as the corresponding salts of the alkali metals or ammonia.

The addition of sulfur dioxide either as such or in the form of sulfurous acid, or as a bisulfite or other salt yielding sulfite ion is made in an amount greater than that needed as an anti-chlor, and has been found to result in a brightening of the pulp by a number of points. Various bleaching aids may be used if desired, as for example magnesium sulfate, sodium silicate, these salts being added to the bleaching bath. However, we have not thus far found them to be necessary, excellent results having been obtained without their aid.

We claim:

1. The method of hypochlorite bleaching of ground wood of the type rich in tannin and color bodies, to yield a ground wood of a brightness at least equal to that which obtains by the hypochlorite bleaching of ground spruce wood, which comprises first extracting therefrom the tannin and color bodies soluble in dilute aqueous caustic alkali solution at temperatures under the boiling point thereof, and then reacting the extracted ground wood with hypochlorite ion in alkaline solution in an amount not substantially in excess of 15% available chlorine based on the dry ground wood.

2. The method of hypochlorite bleaching of ground wood of the type rich in tannin and color bodies, to yield a ground wood of a brightness at least equal to that which obtains by the hypochlorite bleaching of ground spruce wood, which comprises first extracting therefrom the tannin and color bodies soluble in dilute aqueous caustic alkali solution at temperatures under the boiling

point thereof by treating same with a dilute solution of sodium hydroxide in quantity not substantially more than ten per cent. sodium hydroxide based on the dry weight of the pulp, washing the so treated ground wood and then reacting the extracted ground wood with hypochlorite ion in alkaline solution in an amount not substantially in excess of 15% available chlorine based on the dry ground wood.

3. The method of hypochlorite bleaching of oak ground wood to yield a ground wood of a brightness at least equal to that which obtains by the hypochlorite bleaching of ground spruce wood, which comprises first extracting therefrom the tannin and color bodies soluble in dilute aqueous caustic alkali solution at temperatures under the boiling point thereof by treating same with a dilute solution of sodium hydroxide in quantity not substantially more than ten per cent. sodium hydroxide based on the dry weight of the pulp, and then reacting the extracted ground wood with hypochlorite ion in alkaline solution in an amount not substantially in excess of 15% available chlorine based on the dry ground wood.

4. The method according to claim 1, in which the reaction with hypochlorite ion is carried out with a pH in excess of 10.

5. The method of hypochlorite bleaching of ground wood of the type rich in tannin and color bodies, to yield a ground wood of a brightness at least equal to that which obtains by the hypochlorite bleaching of ground spruce wood, which comprises first extracting therefrom the tannin and color bodies soluble in dilute aqueous caustic alkali solution at temperatures under the boiling point thereof, and then reacting the extracted ground wood with hypochlorite ion in an alkaline solution in an amount in excess of ten per cent. but not substantially in excess of fifteen per cent. available chlorine based on the dry ground wood.

DANIEL O. ADAMS.

GEORGE B. HUGHEY.

REFERENCES CITED

45 The following references are of record in the file of this patent:

UNITED STATES PATENTS

| Number    | Name         | Date          |
|-----------|--------------|---------------|
| 200,085   | Patrick      | Feb. 5, 1878  |
| 223,670   | Farrell      | Jan. 20, 1880 |
| 263,797   | Mitscherlich | Sept. 5, 1882 |
| 1,052,675 | Loomis       | Feb. 11, 1913 |
| 1,203,511 | Embree       | Oct. 31, 1916 |
| 1,539,433 | Schorger     | May 26, 1925  |
| 1,843,467 | Traquair     | Feb. 2, 1932  |
| 2,187,016 | Craig        | Jan. 16, 1940 |
| 2,359,891 | Brallier     | Oct. 10, 1944 |

FOREIGN PATENTS

| Number  | Country       | Date          |
|---------|---------------|---------------|
| 101,475 | Great Britain | Oct. 11, 1917 |
| 296,547 | Great Britain | Sept. 6, 1928 |
| 298,333 | Great Britain | Oct. 11, 1928 |

OTHER REFERENCES

65 Bard: "Effect of Tannins . . ." Tech. Assn. Papers, Series XXIV, 1941, pages 199-203, page 203 esp. pertinent.